

Patented July 8, 1947

2,423,692

# UNITED STATES PATENT OFFICE

2,423,692

## NORMAL SECONDARY NONADECYL SULPHATES

Emil E. Dreger, Summit, and John Ross, Ramsey,  
N. J., assignors to Colgate-Palmolive-Peet  
Company, Jersey City, N. J., a corporation of  
Delaware

No Drawing. Original application July 9, 1937,  
Serial No. 152,852. Divided and this applica-  
tion May 26, 1943, Serial No. 488,558

6 Claims. (Cl. 260—459)

1

This invention relates to new materials adapted to function as wetting agents, detergents or the like. More particularly, the invention relates to the utilization of short chain fatty acids, which are not ordinarily satisfactory for the preparation of detergents, wetting agents, and the like, for the production of materials which will function efficiently for these purposes.

The fatty oils that are commonly used in the production of detergent materials almost invariably contain an appreciable percentage of fatty acid esters, the fatty acids of which contain less than 12 carbon atoms. The sodium salts of these fatty acids are of little or no value and, if they are left in the mixture along with the salts of the higher fatty acids, the result is simply a corresponding amount of inactive or inefficient material in the final product. This fact has been recognized and in some instances these lower fatty acids have been removed to make the final product more effective.

The removal of such fatty acids, however, reduces the quantity of the final detergent product that can be produced from a given amount of fatty oil and yields, as a by-product, considerable quantities of these lower fatty acids. For example, about 21% of the fatty acids in coconut oil contains less than 12 carbon atoms, and about 13% of the acids in palm kernel oil also contains less than 12 carbon atoms.

According to the present process, these fatty acids, containing more than 1 and less than 12 carbon atoms and which are almost entirely of the straight chain or normal variety, are reacted in such a way as to form useful, efficient detergents, wetting agents, or the like. Preferably, the fatty acids that are used according to the present process are straight chain fatty acids and have at least 6 and not over 11 carbon atoms.

Briefly, the process of the present invention is accomplished by converting the fatty acids into ketones, usually straight chain ketones since the fatty acids used are generally straight chain fatty acids; thereafter hydrogenating the ketones to form secondary alcohols; and finally sulphating the alcohols to produce secondary alcohol sulphuric acid esters. The acid esters may then be neutralized with lime, ammonia, alkali metal hydroxides or carbonates before use. The process is further described and is claimed in our co-pending application Serial No. 152,852, filed July 9, 1937, now Patent No. 2,321,020, granted June 8, 1943, of which the present application is a division.

The process of the present invention was applied to caproic acid, caprylic acid and capric acid as well as to mixtures of capric and caprylic acids and of all three acids. The individual acids yielded di n-amyl carbinol sulphate salt, di n-heptyl carbinol sulphate salt, and di-n-nonyl

2

carbinol sulphate salt respectively. The mixture of caprylic and capric acid gave a mixture of di n-nonyl carbinol sulphate salt, di n-heptyl carbinol sulphate salt and n-heptyl n-nonyl carbinol sulphate salt. The mixture of all three acids produced in addition to the others n-amyl n-heptyl carbinol sulphate salt and n-amyl n-nonyl carbinol sulphate salt.

The relative wetting and foaming properties 10 of solutions of some of the compounds are compared below, showing the outstanding and unusual efficiency of di n-heptyl carbinol sulphate sodium salt in these respects.

| 15 | Material                                                                                            | Foam, cc.        |                                              | Wetting Time |       |      |
|----|-----------------------------------------------------------------------------------------------------|------------------|----------------------------------------------|--------------|-------|------|
|    |                                                                                                     | 1% Solu-<br>tion | 0.5% in<br>Hard<br>Water,<br>500<br>P. P. M. | 1.0%         | 0.25% | 0.1% |
| 20 | Di-n-heptyl carbinol sul-<br>phate sodium salt<br>$C_7H_{15}O SO_3Na$                               | 500              | 60                                           | 1            | 2     | 10   |
| 25 | n-Heptyl n-nonyl carbinol<br>sulphate sodium salt<br>$C_7H_{15}O SO_3Na$                            | 400              | 20                                           | 2            | 9     | —    |
| 25 | Di-n-nonyl carbinol sul-<br>phate sodium salt<br>$C_9H_{19}O SO_3Na$                                | 275              | 10                                           | 9            | 50    | —    |
| 30 | Mixed sodium salts of car-<br>binol sulphates from<br>mixtures of $C_6$ , $C_8$ , $C_{10}$<br>acids | 350              | 60                                           | 2            | —     | 17   |

The foaming test was conducted by placing 50 cc. of the particular material in a 500 cc. stoppered granulated cylinder at room temperature 35 and shaking the container 20 times in a vertical plane. The volume of the foam was read after allowing the container to stand two minutes.

The wetting test was conducted by comparing the time required by the various solutions to wet 40 a one inch square of unused canvas drill. By placing 100 cc. of the solution to be tested in a beaker, the time required to wet the square of cloth dropped upon the surface of the solution can be readily measured with a stop watch. In 45 most cases the cloth will sink to the bottom as soon as it is thoroughly wet.

Generally the secondary alcohol sulphates prepared by the process should contain at least 11 carbon atoms to be satisfactory as emulsifying 50 and deterging agents. That is, if a single acid is used to prepare the secondary alcohol it should contain at least 6 carbon atoms and, if a mixture of acids is used, the sum of the carbons in their chains should be at least equal to 12 carbon atoms. For example, n-butyric acid (4) and n-caprylic acid (8) will yield along with other sulphates, n-propyl n-heptyl carbinol sulphate salt which has 11 carbon atoms in the compound.

Although the preferred compounds are pre- 55 pared from the straight chain fatty acids con-

taining not less than 6 and not more than 11 carbon atoms, the process is adapted to the use of any straight or branch chain aliphatic monocarboxylic acids other than formic acid, i. e., acetic acid and its higher homologues, whether derived from fatty oils or from any other source, such as the oxidation of petroleum, alcohols and aldehydes, de-esterification of oils, fats and waxes and by organic synthesis.

Mixtures of lauric and n-butyric and of lauric and isobutyric acids were converted into ketones and the pure n-propyl undecyl ketone and iso-propyl undecyl ketone obtained by fractionation. These were reduced to the respective carbinols which were converted into acid sulphates and neutralized.

The following comparison of the wetting and foaming properties of these two isomeric compounds discloses the marked superiority of the straight chain compound as a wetting agent.

- 4
- The present invention is not to be restricted to any specific proportions or manner of procedure beyond the limitation of the appended claims.
- We claim:
5. 1. A normal secondary nonadecyl sulphate.
  2. Di-n-nonyl carbinol sulphate.
  3. A normal secondary nonadecyl sulphate salt.
  4. Di-n-nonyl carbinol sulphate salt.
  10. 5. A normal secondary nonadecyl sulphate sodium salt.
  6. Di-n-nonyl carbinol sulphate sodium salt.

EMIL E. DREGER.  
JOHN ROSS.

#### REFERENCES CITED

The following references are of record in the file of this patent:

#### UNITED STATES PATENTS

|    | Number    | Name            | Date          |
|----|-----------|-----------------|---------------|
|    | 2,027,896 | Bertsch         | Jan. 14, 1936 |
|    | 2,229,649 | Guenther et al. | Jan 28, 1941  |
|    | 2,326,270 | Wernitz         | Aug. 10, 1943 |
| 20 | 2,108,133 | McCall          | Feb. 15, 1938 |
|    | 2,088,019 | Wickert         | July 27, 1937 |

#### FOREIGN PATENTS

|    | Number  | Country       | Date         |
|----|---------|---------------|--------------|
| 30 | 343,872 | Great Britain | Feb. 9, 1931 |

#### OTHER REFERENCES

Messer, "Chem. News," vol. 138, pp. 292-3 (1929).

| Material                                                              | Foam, cc.        |                                              | Wetting Time |       |
|-----------------------------------------------------------------------|------------------|----------------------------------------------|--------------|-------|
|                                                                       | 1% Solu-<br>tion | 0.5% in<br>Hard<br>Water,<br>500<br>P. P. M. | 1%           | 0.25% |
| Isopropyl undecyl carbinol sulphate sodium salt $C_{15}H_{31}OSO_3Na$ | 325              | 115                                          | 13           | 73    |
| n-Propyl undecyl carbinol sulphate sodium salt $C_{15}H_{31}OSO_3Na$  | 300              | 100                                          | 2            | 22    |